

Sept. 17, 1929.

F. A. HAUGHTON

1,728,895

METHOD OF MAKING FIELD RINGS

Filed Oct. 26, 1926

2 Sheets-Sheet 1

Fig. 1.



Fig. 2.



Inventor:

*F. A. Haughton*

Sept. 17, 1929.

F. A. HAUGHTON

1,728,895

METHOD OF MAKING FIELD RINGS

Filed Oct. 26, 1926

2 Sheets-Sheet 2

Fig. 3.



Fig. 4.



Inventor:

*F. A. Haughton*

## UNITED STATES PATENT OFFICE

FRANK A. HAUGHTON, OF SCHENECTADY, NEW YORK, ASSIGNOR TO GENERAL ELECTRIC COMPANY, A CORPORATION OF NEW YORK

## METHOD OF MAKING FIELD RINGS

Application filed October 26, 1926. Serial No. 144,366.

My invention relates to the manufacture of ring-shaped structures and particularly to field rings for direct current dynamo-electric machines. A common practice in the past has been to construct such field rings of gray iron or steel castings, the latter being preferred by reason of their more suitable magnetic properties and greater strength. It not infrequently happens, however, that 5 a casting which appears at first to be perfect proves to be defective after considerable labor has been expended in machining it and must be discarded. Such defective castings are so common and the losses resulting therefrom are so great that the cost of acceptable castings is greatly increased thereby. What perhaps is a more serious objection to the use of castings for magnet frames is the difficulty in obtaining rings having the desired 10 uniformity in magnetic properties inasmuch as hidden defects are likely to exist which are not easily detected. For these and other reasons the use of rolled steel for the field frames of large dynamo-electric machines has 15 been recognized as highly desirable but because of the high cost of frames so made there has been little, if any, inducement to make such a substitution. This high cost is due first, to the cost of the material employed, 20 second, to the cost of labor or special machines or both for shaping the material to the proper form. These considerations are particularly important in the case of machines of large size. 25

It is an object of my invention to provide improved steel rings suitable for the field frames of dynamo-electric machines which are superior to and which may be manufactured at lower costs than the rings now used together with the process of their manufacture. As a result of my invention large economies are obtained both by reason of the material employed and the simple and inexpensive method utilized in working that material, the use of special and expensive tools and highly skilled labor being rendered unnecessary. 40

In accordance with my invention I construct rings of a comparatively cheap form of

rolled steel, namely, "rerolling slabs" or "forging billets" these being the terms generally applied in the trade to the product of the first rolling process to which the steel is subjected in the steel mill after the casting of the ingot. The surface of these slabs, which term will be used hereafter for convenience to apply to both rerolling slabs and forging billets, have a more or less rough and unfinished surface but have magnetic properties which are superior to those of steel castings to the extent that they can be made materially smaller in cross section for the same capacity machine. In utilizing these slabs in accordance with my invention I pass them 55 while at a forging temperature one or more times as may be found necessary through common bending rolls to give them the desired curvature. As a result of this rolling process a slab will be bent uniformly throughout its length with the exception of the two end portions, which as is well known to those skilled in the art, will remain more or less straight. The slab having been given the desired curvature is removed from the bending rolls and the straight or improperly bent 60 end portions are then cut off by means well known to the steel worker. The end faces of the bent sections are then machined to obtain a flat surface and suitable means are 65 provided for securing end to end the ring segments thus formed. Suitable supporting brackets or feet also may be secured to one or more of the ring segments. 70

My invention will be better understood 75 from the following description taken in connection with the accompanying drawing, and its scope will be pointed out in the appended claims. 80

Referring to the drawing, Fig. 1 shows a 85 rerolling slab as it appears when received from the rolling mill; Fig. 2 shows the same slab being bent in the bending rolls; Fig. 3 shows the bent slab after removal from the bending rolls; and Fig. 4 shows a dynamo-electric machine having a split field magnet constructed in accordance with my invention 90 of two such bent slabs, the armature and the bearing supports therefor being omitted. 95

The rerolling slab 1, shown by itself in Fig. 100

1, as has already been pointed out above is the product of the first rolling process to which the ingot is subjected in the steel mill. It is more or less crooked and unshapely and distinctly shows the imprint 2 of the ragging rolls between which it is passed in this first rolling process. The slabs also usually have one or more blisters or other defects on their surfaces which it is the practice of the mill 5 to cut away by hand before further rolling of the slabs. In the present use of the slabs, however, such defects are not objectionable and need not be removed. Slabs are obtained in various sizes in accordance with the sizes 10 of the machines to be constructed, for example, the slab shown in Fig. 1 is about eight and one half inches thick and about twenty-three feet long, weighing approximately seven tons.

20 The slab is first uniformly heated in a suitable furnace to a forging temperature whence it is removed and while hot is passed through common bending rolls. In Fig. 2 I have shown the slab 1 being passed through the 25 bending rolls 3 which are variously constructed and are well known in the art. I have chosen to illustrate bending rolls of a common form but of exceptionally large size comprising a large roll 4 and two cooperating 30 small rolls 5, the large roll being adjustable relative to the small rolls to obtain the desired degree of bend in the material passed therethrough. The slab is passed forward and back through the bending rolls in the 35 usual manner until its curvature corresponds with a template or other gauge. Passage of the slab through the bending rolls also has the effect of partially smoothing out the ragging and other irregularities on the surface of the slab as shown in Figs. 2, 3 and 4 and what 40 remains is an advantage rather than an objection since it provides a better surface to which may cling the putty and paint finish of the machine. The slab is thus given the desired bend throughout the greater portion of 45 its length but its two end portions 6 will remain substantially straight or unbent for a certain distance, as indicated on the drawing. These end portions 6 will be referred to hereafter as unbent inasmuch as they do not have the curvature of the intermediate portion of the ring. If the field ring being constructed 50 is to comprise two ring segments of 180 degrees each, as illustrated by way of example 55 in the drawing, the length of each slab must be sufficient to obtain the 180 degrees of the intermediate or uniformly bent portion plus the unbent end portions. After the bending operation is complete the slab is removed 60 from the bending rolls and the unbent ends 6 are cut off squarely, the line of cut off being indicated by the dotted lines 7 in Fig. 3. In cutting off the ends sufficient material may be 65 left to allow for subsequent machining if necessary to obtain flat end faces. The end

portions which have been cut off while constituting a waste is in reality only a small amount in comparison with the remaining ring segment and has relatively small value being more than offset by the saving in labor 70 and material resulting from this method.

In Fig. 4 I have shown the two ring segments secured together by bolts 9 passing through lugs 10 at the adjacent ends of the ring segments, also the lower ring segment 75 provided with supporting brackets or feet 11. The lugs and feet may be secured to the ring segments in any suitable manner for example by welding and I have found it to be of some 80 advantage to secure the lugs 10 to the ring segments so that the lugs and the end faces of the ring segments may be machined simultaneously whereby a larger area of contact is provided between the adjacent surfaces of the segments. After securing the segments 85 together the ring 12 formed thereby may be machined on its inner surface to which field pole pieces, shown for example at 13 having windings 14, may be attached. The end faces of the field ring may also be machined to 90 which end heads may be secured for supporting the armature, brush holders, etc.

As has been pointed out above the field frames of dynamo-electric machines heretofore have commonly been made of steel castings. As is well known, castings require patterns which in the case of large machines are 95 in themselves costly. Variations in shrinkage and draft requirements of castings necessitate due allowance in the dimensions of the 100 parts and in the making of steel castings moreover it is necessary also to provide large swells and projections for risers. In the finishing process all this excess material must be machined off requiring much time and 105 labor.

By using rerolling slabs a pattern is not required, the ring segments can be formed much closer to size and more nearly circular, no draft allowance need be provided and there 110 are no swells or riser projections to be machined off. Hence there is a decided economy in weight and in cost of machining off surplus metal. As rings formed of rerolling slabs do 115 not contain blow holes, sand holes, scabs, etc. there is no loss due to such defects which are inherent with castings. Moreover such rings are not subject to commutator troubles in the completed machine which sometimes occur where cast frames are used in which hidden 120 defects are present. The magnetic properties of rerolling slabs of low carbon content of say .1 to .2% carbon are very satisfactory as compared with iron or steel castings and experience has shown that frames made from 125 such slabs may be constructed materially lighter in net weight. In the design of machines with cast steel frames a flux density of 75,000 lines per square inch heretofore has been allowed but with frame constructed of 130

rerolling slabs a flux density of 90,000 lines is being regularly employed, due to their greater permeability.

Rerolling slabs having been given only the 5 first rolling and hence subject to a minimum labor cost are the cheapest form of so-called semi-finished steel and can be purchased at the present time for about one quarter of the price of steel castings. This saving in initial 10 cost of material taken together with the economies resulting from the above described method of forming a finished ring from that material has been found in the case of a number of machines to amount to from 30% to 15 40% in factory costs of the finished frames ready for the attachment of poles and other parts.

What I claim as new and desire to secure by Letters Patent of the United States, is,—  
20 1. The method of forming a ring-shaped member from steel slabs which comprises passing the slabs through bending rolls to give them the desired curvature, cutting off the unbent end portions, and joining the bent 25 portions end to end.

2. The method of forming a ring segment from a steel slab which comprises passing the slab through bending rolls to bend only a portion intermediate the ends thereof to the desired curvature and then cutting off the unbent 30 end portions.

3. The method of forming a field ring for a dynamo-electric machine from thick steel slabs which comprises passing the slabs in a 35 heated condition through bending rolls to form ring segments, cutting off the unbent end portions of each segment to form flat end faces and securing the segments together end to end.

40 4. The method of forming a split field ring for a dynamo-electric machine from rerolling slabs which comprises heating the slabs, passing them through bending rolls to form ring segments and to produce a more smooth 45 surface, cutting off the unbent end portions of the segments, machining the end faces and firmly securing the segments together to form a ring.

In witness whereof, I have hereunto set my  
50 hand this 23rd day of October, 1926.

FRANK A. HAUGHTON.